

Patented Apr. 22, 1941

2,239,058

# UNITED STATES PATENT OFFICE

2,239,058

## HARD METAL ALLOY

Robert W. Schlumpf, Houston, Tex., assignor to  
Hughes Tool Company, Houston, Tex., a cor-  
poration of Delaware

No Drawing. Application May 20, 1940,  
Serial No. 336,135

2 Claims. (Cl. 75—126)

This invention relates to a hard wear resisting alloy such as is applied to surfaces of tools and the like which are subject to wear and abrasion in use.

It is an object of the invention to provide a hard alloy which is also tough and resistant to shock stresses of mechanical or thermal origin and thus not easily broken or shattered when employed on scrapers, cutters, bearings, nozzles, and the like.

I desire to provide hard facing members which can be precast and fixed in position upon tools and devices by copper brazing.

My tough and wear resistant alloy has, as its principal hard ingredient about 16% of tungsten. This substance is fused together with other metals which serve to render the resulting alloy particularly tough and not liable to shatter.

The elements making up my improved alloy may vary somewhat as to proportions. The following table shows the metals in the proportions found most effective:

|                                      | Per cent       |
|--------------------------------------|----------------|
| Carbon                               | 1.00 to 4.00   |
| Manganese                            | 0.50 to 2.00   |
| Silicon                              | 0.50 to 2.00   |
| Chromium                             | 2.00 to 6.00   |
| Molybdenum                           | 3.50 to 6.50   |
| Tungsten                             | 14.00 to 18.00 |
| Iron, balance to make up 100% in all |                |

These metals may be fused together at a temperature of about 2300° to 2400° F.

I contemplate applying this alloy by first casting the alloy in the shape desired whether in plates, tubes, inserts, or the like, and then fixing the precast members in position by brazing; using copper or copper compounds for the purpose.

The hard metal alloy produced by my formula is not only exceedingly hard, but is resistant to fracture which is liable to result from shocks, thermal stresses and the like. It thus overcomes some serious objections to other common hard facing alloys now in use.

What I claim as new is:

1. A wear resisting alloy comprising in combination:

|                               | Per cent       |
|-------------------------------|----------------|
| Carbon                        | 1.00 to 4.00   |
| Manganese                     | 0.50 to 2.00   |
| Silicon                       | 0.50 to 2.00   |
| Chromium                      | 2.00 to 6.00   |
| Molybdenum                    | 3.50 to 6.50   |
| Tungsten                      | 14.00 to 18.00 |
| Balance iron to make up 100%. |                |

2. A wear resisting alloy made up of the following elements fused together in proportions approximately as set forth below:

Carbon 1½%; manganese and silicon each from 0.50% to 2.00%; chromium and molybdenum each 5.00%; tungsten from 14.00% to 18.00%, and iron to make 100%.

ROBERT W. SCHLUMPF.